# EUROPEAN PATENT SPECIFICATION

(11) **EP 3 770 295 B1**
(45) Date of publication and mention of the grant of the patent: **16.08.2023**
(21) Application number: 19847997.4
(22) Date of filing: 06.09.2019
(51) Int. Cl.: C23C 2/12, C22C 38/02, C22C 38/04, C22C 38/06, C22C 38/28, C22C 38/32, C21D 1/18, C21D 1/673, C21D 1/76, C21D 6/00, C21D 7/13, C21D 9/48, C22C 38/38, C23C 2/28, C23C 28/02, B21D 22/02

(54) **MANUFACTURING METHOD FOR HOT STAMPING COMPONENT HAVING ALUMINIUM-SILICON ALLOY COATING**
VERFAHREN ZUR HERSTELLUNG EINES HEISSPRÄGE-BAUTEILS MIT ALUMINIUM-SILIZIUM-LEGIERUNGSBESCHICHTUNG
PROCÉDÉ DE FABRICATION D'UN COMPOSANT D'ESTAMPAGE Á CHAUD AYANT UN REVÊTEMENT EN ALLIAGE ALUMINIUM-SILICIUM

(30) Priority: 08.08.2018 CN 201810896744; 06.09.2018 CN 201811035118
(43) Date of publication of application: 27.01.2021
(73) Proprietor: BAOSHAN IRON & STEEL CO., LTD., Shanghai 201900 (CN)
(72) Inventor: TAN, Ning, Shanghai 201900 (CN); FU, Jiang, Shanghai 201900 (CN); HONG, Jiyao, Shanghai 201900 (CN); FANG, Xuehua, Shanghai 201900 (CN)
(74) Representative: Maiwald GmbH
(86) International application number: PCT/CN2019/104708
(87) International publication number: WO 2020/030200

(56) References cited:
- EP-A1- 3 070 187
- CN-A- 101 117 697
- CN-A- 102 300 707
- CN-A- 102 605 308
- CN-A- 105 886 750
- CN-A- 106 466 697
- CN-A- 106 734 470
- CN-A- 106 995 875
- CN-A- 109 518 114
- US-A- 4 714 500
- US-A1- 2011 056 594
- SINGH JHAJJ KAMALPREET: "Heat Transfer Modeling of Roller Hearth and Muffle Furnace", THESIS UNIVERSITY OF WATERLOO, 1 January 2015 (2015-01-01), pages 1-53, XP055808280, Retrieved from the Internet: URL:https://core.ac.uk/download/pdf/144148 558.pdf>
- N/a: "Advancements in furnace design improve hot stamping", Stamping Journal, 28 February 2017 (2017-02-28), pages 1-7, XP055883524, Retrieved from the Internet: URL:https://www.thefabricator.com/stamping journal/article/stamping/advancements-in-f urnace-design-improve-hot-stamping [retrieved on 2022-01-25]
- N/a: "ASTM standard A 463/A463 M", , 10 August 2016 (2016-08-10), pages 1-7, XP055883519, Retrieved from the Internet: URL:https://www.astm.org/a0463_a0463m-15r2 0e01.html [retrieved on 2022-01-25]
- N/a: "Stress-Strain Curves - Usibor 1500 treated", , 31 December 2016 (2016-12-31), pages 1-5, XP055883494, Retrieved from the Internet: URL:https://automotive.arcelormittal.com/f iles/Usibor1500--3a82a9aa69487763bbbba1a96 0151cc0.pdf [retrieved on 2022-01-25]

## Description

### Technical Field

The present invention relates to manufacturing technology of hot stamping components, in particular to a manufacturing method of a hot stamping component having an aluminum-silicon alloy coating and a hot stamping component.

### Background Art

Lightweight and emission reduction are the main development trends of the automotive industry. High strength of automotive parts is finally achieved by heat treatment for changing the microstructure of the materials when using relatively low-strength materials. This hot forming technique realizes the improvement of forming level of automotive parts and guarantees the high strength properties. Compared with uncoated hot stamping products, the one that has an aluminum-silicon coating has a good thickness and dimensional accuracy, good corrosion resistance and welding performance. The proportion of hot stamping steels with an aluminum-silicon coating accounts for 70% of the hot stamping steels currently in use, and it will get higher and higher for the foreseeable future.

Chinese patent CN101583486B discloses a method of coated stamping products, including the temperature and time of stamping, wherein the heating rate from room temperature to 700 °C is 4-12 °C/s, which aims at ensuring the spot welding performance of stamping components.

Chinese patent CN102300707B further discloses a heating method of coated hot stamping components, specifically discloses the heating rate under melting temperature, the holding time under austenitizing temperature, etc. However, considering the efficiency and production cycle time of the heat treatment furnace during use, users find that this heating method still could not solve the problem of adhesion to the roller and nodulation by aluminum-silicon coating, which causes problems such as the decrease in service life of heat treatment furnace roller and peeling of coating of hot stamping components.

Sigh Jhali Kamalpreet: "Heat Transfer Modeling of Roller Hearth and Muffle Furnace", Thesis, University of Waterloo, 1 January 2015 (2015-01-01), pages 1-53, XP055808280 discloses a hot forming die quenching method.

US 2011/056594 A1 discloses a process for producing a component from a steel product coated with a protective Al-Si coating.

### Summary of the Invention

The purpose of the present invention is to provide a manufacturing method of a hot stamping component having an aluminum-silicon alloy coating and a hot stamping component, which can not only effectively solve the problem of adhesion to the roller by aluminum-silicon coating, reduce the nodulation probability of the heat treatment furnace roller and improve the service life of the roller, but can also ensure the integrity of the coating of the hot stamping component and the mechanical properties, welding performance, coating performance and corrosion resistance of the component.

To achieve the above purpose, the technical solutions of the present invention are defined in the appended claims.

According to a first aspect, the present invention relates to a manufacturing method of a hot stamping component having an aluminum-silicon alloy coating, comprising the following steps: machining a steel plate coated with an aluminum-silicon alloy coating into a blank having a shape required for a part; conducting heat treatment and hot stamping of the blank; wherein, in the heat treatment of the blank, the blank is put into a heat treatment furnace for austenitizing heat treatment, and the heat treatment process of the blank comprises a first heating and holding stage, a second heating and holding stage, and a third heating and holding stage;
and wherein:
when the thickness of the steel plate coated with an aluminum-silicon alloy coating is less than 1.5 mm,
in the first heating and holding stage, the temperature and time of heating and holding lie within a graph ABCD, the graph ABCD represents the ranges of temperature and time defined by coordinates of A (750 °C, 30 s), B (750 °C, 90 s), C (870 °C, 90 s) and D (870 °C, 30 s); and
in the second heating and holding stage, the temperature and time of heating and holding lie within a graph EFGH, the graph EFGH represents the ranges of temperature and time defined by coordinates of E (875 °C, 60 s), F (875 °C, 240 s), G (930 °C, 150 s) and H (930 °C, 30 s); and
in the third heating and holding stage, the temperature and time of heating and holding lie within a graph IJKL, the graph IJKL represents the ranges of temperature and time defined by coordinates of I (935 °C, 60 s), J (935 °C, 240 s), K (955 °C, 180 s) and L (955 °C, 30 s);
when the thickness of steel plate coated with an aluminum-silicon alloy coating is 1.5 mm or more,
in the first heating and holding stage, the temperature and time of heating and holding lie within a graph A'B'C'D', the graph A'B'C'D' represents the ranges of temperature and time defined by coordinates of A' (750 °C, 30 s), B' (750 °C, 90 s), C' (890 °C, 90 s) and D' (890 °C, 30 s); and
in the second heating and holding stage, the temperature and time of heating and holding lie within a graph E'F'G'H', the graph E'F'G'H' represents the ranges of temperature and time defined by coordinates of E' (895 °C, 90 s), F' (895 °C, 270 s), G' (940 °C, 210 s) and H' (940 °C, 60 s); and
in the third heating and holding stage, the temperature and time of heating and holding lie within a graph I'J'K'L', the graph I'J'K'L' represents the ranges of temperature and time defined by coordinates of I' (945 °C, 60 s), J' (945 °C, 240 s), K' (955 °C, 180 s) and L' (955 °C, 30 s).

Preferably, in the heat treatment process of the blank, the temperature increases stepwise in the order of the first, second, and third heating and holding stages or the temperatures in the first, second, and third heating and holding stages are set to be certain temperatures.

For example, for the steel plate having a thickness of 1.2 mm and an aluminum-silicon alloy coating, the heat treatment process can be as follows: the temperature and time of the first heating and holding stage are 800 °C and 60 s, respectively; and the temperature and time of the second heating and holding stage are 930 °C and 120 s, respectively; and the temperature and time of the third heating and holding stage are 940 °C and 60 s, respectively. The heat treatment process can also be as follows: multiple temperatures, for example 770 °C for 40 s, 820 °C for 30 s and 770 °C for 50 s are set in the first heating and holding stage; and multiple temperatures, for example 900 °C for 60 s and 930 °C for 60 s are set in the second heating and holding stage; and multiple temperatures, for example 935 °C for 60 s and 940 °C for 60 s are set in the third heating and holding stage.

Preferably, the time of the heat treatment process of the blank is not less than 150 s and not more than 600 s. Within this time range, the blank after heat treatment has high surface quality, good coating performance, and good welding performance.

Preferably, a heat treatment furnace is used in the heat treatment process of the blank. The oxygen content in the furnace's atmosphere is not less than 15% and the dew point in the furnace is not higher than -5 °C. The final hot stamping component has a low hydrogen content and an excellent resistance to delayed cracking.

Preferably, in the hot stamping process, the heat-treated blank is quickly transferred to a mold for stamping, the transfer time is 4-12 seconds, and the blank is in a temperature of not lower than 600°C before being fed into the mold; the mold is cooled before stamping to ensure that the surface temperature of the mold before stamping is lower than 100 °C, and the cooling rate of the blank is greater than 30 °C/s. The microstructure of the hot stamping component obtained through the above process is mainly martensite or bainite, and the hot stamping component has excellent mechanical properties and meets the requirements for use.

Preferably, in the hot stamping process, the steel plate coated with an aluminum-silicon alloy coating comprises a substrate and an aluminum-silicon alloy coating on at least one surface of the substrate, and the substrate comprises the following composition in percentage by weight: C: 0.04-0.8%, Si<1.2%, Mn: 0.1-5%, P<0.3%, S<0.1%, Al<0.3%, Ti<0.5%, B<0.1%, Cr<3% and the rest being Fe and inevitable impurities.

Preferably, the aluminum-silicon alloy coating comprises the following composition in percentage by weight: Si: 4-14%, Fe: 0-4%, and the balance being Al and inevitable impurities. By adopting the above-mentioned silicon alloy coating composition, the obtained alloy coating has a uniform and thin thickness, the coating has good adhesion and good machinability.

Preferably, the average weight of the aluminum-silicon alloy coating is 58-105 g/m² on one side; more preferably, the average weight of the aluminum-silicon alloy coating is 72-88 g/m² on one side. By controlling the average weight of the aluminum-silicon alloy coating within the range, the final hot stamping component has a uniform appearance and color (no color difference), good coating performance, and good welding performance.

In addition, the aluminum-silicon alloy coating of the hot stamping component obtained by the manufacturing method of the present invention comprises a surface alloy layer and a diffusion layer, and the ratio of the thickness of the diffusion layer to the thickness of the aluminum-silicon alloy coating is 0.08-0.5. The final hot stamping component has uniform appearance and color, good coating performance and good welding performance.

Specifically, the aluminum-silicon alloy coating comprises two layers, the one that is in contact with the substrate is a diffusion layer. During the heat treatment process, Al in the aluminum-silicon alloy coating and Fe of the substrate further diffuse to form the diffusion layer. Al in the aluminum-silicon alloy coating and Fe of the substrate are alloyed to form a surface alloy layer. In the component after hot stamping, the ratio of the thickness of the diffusion layer to the total thickness of the aluminum-silicon alloy coating (including the diffusion layer and the surface alloy layer) is 0.08-0.5.

The hot stamping component formed with the method of the present invention has a yield strength of 400-1300 MPa, a tensile strength of 500-2000 MPa, and an elongation of 4% or more.

Preferably, the elongation of the hot stamping component according to the present invention is 4 to 20%.

During the heat treatment process of the hot stamping component, no coating melts and adheres to the roller, the coating is complete and has a good adhesion, and there is no significant peeling off the surface.

For the hot stamping component, no coating peels off, the surface roughness meets the requirements, and the ratio of the thickness of the diffusion layer to the thickness of the coating is between 0.08 and 0.5. After electrophoretic coating, the coating film is complete and the coating film adhesion is evaluated as grade 0 or higher.

For the hot stamping component, the thickness of the diffusion layer and the thickness of the coating meet the requirements, the ratio of the thickness of the diffusion layer to the thickness of the coating is between 0.08 and 0.5, and the spot welding performance is excellent with all the spot welding range being 2KA or above.

During the heat treatment process, the coating on the hot stamping component can well meet the diffusion of the coating and the austenitization of the substrate, and the melting and adhesion to the roller of the coating can be avoided, thereby obtaining the hot stamping component with good coating performance and substrate performance.

Specifically, the melting point of Al-Si alloy of the aluminum-silicon alloy coating is between 580 and 600 °C, the austenitizing temperature of the steel plate is 840 °C or above, the aluminum-silicon alloy coating will melt during the heat treatment process, and adhere to the furnace roller. Meanwhile, Al in the coating and Fe of the substrate will diffuse to form an Fe-Al alloy which has a strong heat resistance and a high melting temperature, and will not cause adhesion to the furnace roller. In the present invention, by controlling dwell time of the aluminum-silicon coating in the heating process and in the heating and holding stages, the melting of the aluminum-silicon alloy coating, the adhesion of the coating to the heat treatment furnace roller and the nodulation of the furnace roller are avoided as much as possible. And according to the production cycle time, by ensuring the coating to reach an appropriate alloying degree, obtaining a suitable thickness of the coating and of the diffusion layer, and the surface quality of the coating, the welding performance and coating performance of the component are guaranteed.

The beneficial effects of the present invention are as follows:
By designing the heat treatment process of the blank, the adhesion of the aluminum-silicon alloy coating to the heat treatment furnace roller is reduced, the occurrence rate of nodulation of the heat treatment furnace roller is reduced, and the maintenance cycle and service life of the roller are extended.

Moreover, the heat treatment process of the blank according to the present invention can improve the surface quality of the stamping component and prevent the coating from peeling off during the heat treatment process.

In addition, the heat treatment process of the blank according to present invention adopts a stepwise heating mode, fully considers the characteristics of the aluminum-silicon alloy coating, and appropriately adjusts the temperature and time according to the thickness of the blank, so that the energy can be effectively used and a good energy saving effect is achieved.

### Brief Description of the Drawings

Figure 1 shows a surface of the hot stamping component with an aluminum-silicon alloy coating prepared in Comparative Example 1.
Figure 2 shows a surface of the hot stamping component with an aluminum-silicon alloy coating prepared in Example 1 of the present invention.
Figure 3 is a cross-sectional view of the hot stamping component with an aluminum-silicon alloy coating prepared in Example 1 of the present invention.
Figure 4 is a schematic diagram of the temperature and time ranges of heating and temperature in the first to the third heating and holding stages of the heat treatment process (three-stage heating and holding) of the blank according to the present invention (in the case of the steel plate thickness < 1.5 mm).
Figure 5 is a schematic diagram of the temperature and time ranges of heating and holding in the first to the third heating and holding stages of the heat treatment process (three-stage heating and holding) of the blank according to the present invention (in the case of the steel plate thickness ≥1.5mm).
Figure 6 is a schematic diagram of the temperature and time ranges of heating and holding in the first and the third heating and holding stages of the heat treatment process (two-stage heating and holding) of the blank not according to the present invention.

### Detailed Description

The present invention is further described below with reference to Examples and Figures.

Table 1 shows the compositions of the substrates of the steel plates in Examples of the present invention; Table 2 shows the manufacturing processes and properties of the hot stamping components in Examples of the present invention. Examples 4 and 8 are not according to the present invention.

### Example 1

A substrate with a thickness of 1.2 mm was subjected to hot dip aluminum plating at 650 °C, the composition of the plating bath is 8% of Si and 2.3% of Fe, with the rest being Al and inevitable impurities. The steel plate coated with the aluminum-silicon alloy coating was continuously blanked into a blank with a certain shape. The blank was subjected to a heat treatment, and the specific parameters of the heat treatment are shown in Table 2. The appearance of the obtained hot stamping component is shown in Figure 2. The cross-sectional microstructure of the aluminum-silicon alloy coating is shown in Figure 3. The aluminum-silicon alloy coating comprises a surface alloy layer and a diffusion layer, and the ratio of the thickness of the diffusion layer to the thickness of the aluminum-silicon alloy coating is 0.25.

### Example 2

A substrate with a thickness of 0.9 mm was subjected to hot dip aluminum plating at 660 °C, the composition of the plating bath is 9% of Si and 2.5% of Fe, with the rest being Al and inevitable impurities. The steel plate coated with the aluminum-silicon alloy coating was continuously blanked into a blank with a certain shape. The blank was subjected to a heat treatment, and the specific parameters of the heat treatment are shown in Table 2. The ratio of the thickness of the diffusion layer to the thickness of the aluminum-silicon alloy coating is 0.3.

### Example 3

A substrate with a thickness of 1.0 mm was subjected to hot dip aluminum plating at 660 °C, the composition of the plating bath is 8.5% of Si and 2.5% of Fe, with the rest being Al and inevitable impurities. The steel plate coated with the aluminum-silicon alloy coating was continuously blanked into a blank with a certain shape. The blank was subjected to a heat treatment. The ratio of the thickness of the diffusion layer to the thickness of the aluminum-silicon alloy coating is 0.15.

### Example 4

A substrate with a thickness of 1.1 mm was subjected to hot dip aluminum plating at 680 °C, the composition of the plating bath is 9.5% of Si and 2.5% of Fe, with the rest being Al and inevitable impurities. The steel plate coated with the aluminum-silicon alloy coating was continuously blanked into a blank with a certain shape. The blank was subjected to a heat treatment. The ratio of the thickness of the diffusion layer to the thickness of the aluminum-silicon alloy coating is 0.28.

### Example 5

A substrate with a thickness of 1.2 mm was subjected to hot dip aluminum plating at 680 °C, the composition of the plating bath is 8.8% of Si and 2.4% of Fe, with the rest being Al and inevitable impurities. The steel plate coated with the aluminum-silicon alloy coating was continuously blanked into a blank with a certain shape. The blank was subjected to a heat treatment. The ratio of the thickness of the diffusion layer to the thickness of the aluminum-silicon alloy coating is 0.35.

### Example 6

A substrate with a thickness of 1.5 mm was subjected to hot dip aluminum plating at 680 °C, the composition of the plating bath is 8.8% of Si and 2.4% of Fe, with the rest being Al and inevitable impurities. The steel plate coated with the aluminum-silicon alloy coating was continuously blanked into a blank with a certain shape. The blank was subjected to a heat treatment. The ratio of the thickness of the diffusion layer to the thickness of the aluminum-silicon alloy coating is 0.35.

### Example 7

A substrate with a thickness of 1.6 mm was subjected to hot dip aluminum plating at 680 °C, the composition of the plating bath is 8.8% of Si and 2.4% of Fe, with the rest being Al and inevitable impurities. The steel plate coated with the aluminum-silicon alloy coating was continuously blanked into a blank with a certain shape. The blank was subjected to a heat treatment. The ratio of the thickness of the diffusion layer to the thickness of the aluminum-silicon alloy coating is 0.3.

### Example 8

A substrate with a thickness of 1.8 mm was subjected to hot dip aluminum plating at 680 °C, the composition of the plating bath is 8.8% of Si and 2.4% of Fe, with the rest being Al and inevitable impurities. The steel plate coated with the aluminum-silicon alloy coating was continuously blanked into a blank with a certain shape. The blank was subjected to a heat treatment. The ratio of the thickness of the diffusion layer to the thickness of the aluminum-silicon alloy coating is 0.35.

### Example 9

A substrate with a thickness of 2.0 mm was subjected to hot dip aluminum plating at 680 °C, the composition of the plating bath is 8.8% of Si and 2.4% of Fe, with the rest being Al and inevitable impurities. The steel plate coated with the aluminum-silicon alloy coating was continuously blanked into a blank with a certain shape. The blank was subjected to a heat treatment. The ratio of the thickness of the diffusion layer to the thickness of the aluminum-silicon alloy coating is 0.4.

**Table 1 Composition of the substrate of the steel in percentage by weight (wt %)**

| Examples | C | Si | Mn | P | S | Al | Ti | B | Cr |
|---|---|---|---|---|---|---|---|---|---|
| 1 | 0.22 | 0.10 | 2.90 | 0.059 | 0.038 | 0.09 | 0.090 | 0.031 | 0.150 |
| 2 | 0.10 | 0.02 | 0.8 | 0.018 | 0.007 | 0.08 | 0.001 | 0.001 | 0.003 |
| 3 | 0.20 | 0.23 | 1.19 | 0.015 | 0.040 | 0.08 | 0.027 | 0.005 | 0.200 |
| 4 | 0.39 | 0.36 | 3.00 | 0.044 | 0.030 | 0.07 | 0.050 | 0.006 | 0.300 |
| 5 | 0.08 | 0.05 | 0.70 | 0.02 | 0.010 | 0.05 | 0.002 | 0.002 | 0.220 |
| 6 | 0.25 | 0.40 | 2.30 | 0.059 | 0.038 | 0.09 | 0.090 | 0.031 | 0.150 |
| 7 | 0.12 | 0.20 | 0.90 | 0.018 | 0.007 | 0.08 | 0.001 | 0.001 | 0.003 |
| 8 | 0.30 | 0.30 | 1.70 | 0.015 | 0.040 | 0.08 | 0.027 | 0.005 | 0.200 |
| 9 | 0.50 | 0.36 | 3.00 | 0.044 | 0.030 | 0.07 | 0.050 | 0.006 | 0.300 |
| Comparative Example | 0.22 | 0.10 | 2.90 | 0.059 | 0.038 | 0.09 | 0.090 | 0.031 | 0.150 |

**Table 2**

| Examples | thickness of the steel plate with coating (mm) | the first heating and holding stage | | the second heating and holding stage | | the third heating and holding stage | | the ratio of thickness of alloy layer to thickness of the surface layer |
|---|---|---|---|---|---|---|---|---|
| | | temperatu re (°C) | time of heating and holding (s) | temperatu re (°C) | time of heating and holding (s) | temperatu re (°C) | time of heating and holding (s) | |
| 1 | 1.2 | 750 | 85 | 880 | 100 | 935 | 100 | 0.25 |
| 2 | 0.9 | 770 | 90 | 890 | 60 | 935 | 60 | 0.30 |
| 3 | 1.0 | 790 | 60 | 900 | 130 | 940 | 180 | 0.15 |
| 4 | 1.1 | 800 | 70 | - | - | 950 | 250 | 0.28 |
| 5 | 1.2 | 850 | 55 | 920 | 150 | 950 | 100 | 0.35 |
| 6 | 1.5 | 760 | 90 | 900 | 100 | 945 | 100 | 0.35 |
| 7 | 1.6 | 790 | 80 | 910 | 170 | 945 | 150 | 0.30 |
| 8 | 1.8 | 830 | 70 | - | - | 950 | 230 | 0.35 |
| 9 | 2.0 | 880 | 60 | 930 | 200 | 950 | 80 | 0.40 |
| Comparative Example | 1.2 | - | - | - | - | 945 | 150 | 0.05 |

Figure 1 shows the surface of the hot stamping component in Comparative Example. The aluminum-silicon coating surface melts, which causes the coating to adhere to the roller.

Figure 2 shows the surface of the hot stamping component in Example 1 of the present invention. The aluminum-silicon alloy coating surface shows no sign of melting, and the alloying is sufficient.

Figure 3 is a cross-sectional view of the coating of the hot stamping component in Example 1 of the present invention. It can be seen from the Figure that the aluminum-silicon alloy coating comprises two layers, i.e. a surface alloy layer and a diffusion layer. The ratio of the thickness of the diffusion layer to the thickness of the aluminum-silicon alloy coating is about 0.25. The substrate mainly consists of martensite.

Figure 4 shows the ranges of the first, the second and the third heating and holding stages when the thickness of the steel plate coated with an aluminum-silicon alloy coating according to the present invention is less than 1.5 mm. The temperature and time of heating and holding in the first heating and holding stage lie within a graph ABCD, the temperature and time of heating and holding in the second heating and holding stage lie within a graph EFGH, and the temperature and time of heating and holding in the third heating and holding stage lie within a graph IJKL.

Figure 5 shows the ranges of the first, the second and the third heating and holding stages when the thickness of the steel plate coated with an aluminum-silicon alloy coating according to the present invention is 1.5 mm or more. The temperature and time of heating and holding in the first heating and holding stage lie within a graph A'B'C'D', the temperature and time of heating and holding in the second heating and holding stage lie within a graph E'F'G'H', and the temperature and time of heating and holding in the third heating and holding stage lie within a graph I'J'K'L'.

Figure 6 is a schematic diagram of the temperature and time ranges of heating and holding in the first and the third heating and holding stages of the heat treatment process (two-stage heating and holding) of the blank not according to the present invention, the heating and holding time in the second heating and holding stage is zero, which forms a two-stage heating and holding.

When the thickness of the steel plate coated with an aluminum-silicon alloy coating is less than 1.5 mm, the temperature and time of heating and holding in the first heating and holding stage lie within a graph abcd, and the temperature and time of heating and holding in the third heating and holding stage lie within a graph ijkl.

When the thickness of the steel plate coated with an aluminum-silicon alloy coating is 1.5 mm or more, the temperature and time of heating and holding in the first heating and holding section lie within a graph a'b'c'd', and the temperature and time of heating and holding in the third heating and holding stage lie within a graph i'j'k'l'.

## Claims

1. A manufacturing method of a hot stamping component having an aluminum-silicon alloy coating, comprising the following steps: machining a steel plate coated with an aluminum-silicon alloy coating into a blank having a shape required for a part; conducting heat treatment and hot stamping of the blank;
wherein, in the heat treatment of the blank, the blank is put into a heat treatment furnace for austenitizing heat treatment, and the heat treatment process of the blank comprises a first heating and holding stage, a second heating and holding stage, and a third heating and holding stage;
and wherein:
when the thickness of the steel plate coated with an aluminum-silicon alloy coating is less than 1.5 mm,
in the first heating and holding stage, the temperature and time of heating and holding lie within a graph ABCD, the graph ABCD represents the ranges of temperature and time defined by coordinates of A (750 °C, 30 s), B (750 °C, 90 s), C (870 °C, 90 s) and D (870 °C, 30 s); and
in the second heating and holding stage, the temperature and time of heating and holding lie within a graph EFGH, the graph EFGH represents the ranges of temperature and time defined by coordinates of E (875 °C, 60 s), F (875 °C, 240 s), G (930 °C, 150 s) and H (930 °C, 30 s); and
in the third heating and holding stage, the temperature and time of heating and holding lie within a graph IJKL, the graph IJKL represents the ranges of temperature and time defined by coordinates of I (935 °C, 60 s), J (935 °C, 240 s), K (955 °C, 180 s) and L (955 °C, 30 s);
when the thickness of the steel plate coated with an aluminum-silicon alloy coating is 1.5 mm or more,
in the first heating and holding stage, the temperature and time of heating and holding lie within a graph A'B'C'D', the graph A'B'C'D' represents the ranges of temperature and time defined by coordinates of A' (750 °C, 30 s), B' (750 °C, 90 s), C' (890 °C, 90 s) and D' (890 °C, 30 s); and
in the second heating and holding stage, the temperature and time of heating and holding lie within a graph E'F'G'H', the graph E'F'G'H' represents the ranges of temperature and time defined by coordinates of E' (895 °C, 90 s), F' (895 °C, 270 s), G' (940 °C, 210 s) and H' (940 °C, 60 s); and
in the third heating and holding stage, the temperature and time of heating and holding lie within a graph I'J'K'L', the graph I'J'K'L' represents the ranges of temperature and time defined by coordinates of I' (945 °C, 60 s), J' (945 °C, 240 s), K' (955 °C, 180 s) and L' (955 °C, 30 s).

2. The manufacturing method of a hot stamping component having an aluminum-silicon alloy coating as claimed in claim 1, wherein in the heat treatment process of the blank, the temperature increases stepwise in the order of the first, second, and third heating and holding stages or the temperatures in the first, second, and third heating and holding stages are set to be certain temperatures.

3. The manufacturing method of a hot stamping component having an aluminum-silicon alloy coating as claimed in claim 1, wherein the time of the heat treatment process of the blank is not less than 150 s and not more than 600 s.

4. The manufacturing method of a hot stamping component having an aluminum-silicon alloy coating as claimed in claim 1, wherein a heat treatment furnace is used in the heat treatment process of the blank, the oxygen content in the furnace's atmosphere is not less than 15%, and the dew point in the furnace is not higher than -5 °C.

5. The manufacturing method of a hot stamping component having an aluminum-silicon alloy coating as claimed in claim 1, wherein in the hot stamping process, the heat-treated blank is quickly transferred to a mold for stamping, the transfer time is 4-12 seconds, and the blank is in a temperature of not lower than 600 °C before being fed into the mold; the mold is cooled before stamping to ensure that the surface temperature of the mold before stamping is lower than 100 °C, and the cooling rate of the blank is greater than 30 °C/s.

6. The manufacturing method of a hot stamping component having an aluminum-silicon alloy coating as claimed in claim 1, wherein the steel plate coated with an aluminum-silicon alloy coating comprises a substrate and an aluminum-silicon alloy coating on at least one surface of the substrate, and the substrate comprises the following composition in percentage by weight: C: 0.04-0.8%, Si<1.2%, Mn: 0.1-5%, P<0.3%, S<0.1%, Al<0.3%, Ti<0.5%, B<0.1%, Cr<3%, and the rest being Fe and inevitable impurities.

7. The manufacturing method of a hot stamping component having an aluminum-silicon alloy coating as claimed in claim 6, wherein the aluminum-silicon alloy coating comprises the following composition in percentage by weight: Si: 4-14%, Fe: 0-4%, and the balance being Al and inevitable impurities.

8. The manufacturing method of a hot stamping component having an aluminum-silicon alloy coating as claimed in claim 6 or 7, wherein the average weight of the aluminum-silicon alloy coating is 58-105 g/m² on one side.

9. The manufacturing method of a hot stamping component having an aluminum- silicon alloy coating as claimed in claim 6 or 7, wherein the average weight of the aluminum-silicon alloy coating is 72-88 g/m² on one side.

## Patentansprüche

1. Verfahren zur Herstellung eines Heißpräge-Bauteils mit einer Aluminium-Silizium-Legierungsbeschichtung, umfassend die folgenden Schritte: Bearbeiten einer mit einer Aluminium-Silizium-Legierungsbeschichtung beschichteten Stahlplatte zu einem Rohling mit einer für ein Teil erforderlichen Form; Durchführen einer Wärmebehandlung und Heißprägen des Rohlings;
wobei bei der Wärmebehandlung des Rohlings der Rohling zur Austenitisierungswärmebehandlung in einen Wärmebehandlungsofen eingebracht wird und der Wärmebehandlungsprozess des Rohlings eine erste Erhitzungs- und Haltestufe, eine zweite Erhitzungs- und Haltestufe und eine dritte Erhitzungs- und Haltestufe umfasst;
und wobei:
wenn die Dicke der mit einer Aluminium-Silizium-Legierung beschichteten Stahlplatte weniger als 1,5 mm beträgt,
in der ersten Erhitzungs- und Haltestufe die Temperatur und die Zeit des Erhitzens und Haltens innerhalb eines Graphen ABCD liegen, wobei der Graph ABCD die Bereiche von Temperatur- und Zeitbereiche darstellt, die durch die Koordinaten A (750 °C, 30 s), B (750 °C, 90 s), C (870 °C, 90 s) und D (870 °C, 30 s) definiert sind; und
in der zweiten Erhitzungs- und Haltestufe die Temperatur und die Zeit des Erhitzens und Haltens innerhalb eines Graphen EFGH liegen, wobei der Graph EFGH die Temperatur- und Zeitbereiche darstellt, die durch die Koordinaten E (875 °C, 60 s), F (875 °C, 240 s), G (930 °C, 150 s) und H (930 °C, 30 s) definiert sind; und
in der dritten Erhitzungs- und Haltestufe die Temperatur und die Zeit des Erhitzen und Haltens innerhalb eines Graphen IJKL liegen, wobei der Graph IJKL die Temperatur- und Zeitbereiche darstellt, die durch die Koordinaten I (935 °C, 60 s), J (935 °C, 240 s), K (955 °C, 180 s) und L (955 °C, 30 s) definiert sind;
wenn die Dicke der mit einer Aluminium-Silizium-Legierung beschichteten Stahlplatte 1,5 mm oder mehr beträgt,
in der ersten Erhitzungs- und Haltestufe die Temperatur und die Zeit des Erhitzens und Haltens innerhalb eines Graphen A'B'C'D' liegen, wobei der Graph A'B'C'D' die Temperatur- und Zeitbereiche darstellt, die durch die Koordinaten A' (750 °C, 30 s), B' (750 °C, 90 s), C' (890 °C, 90 s) und D' (890 °C, 30 s) definiert sind; und
in der zweiten Erhitzungs- und Haltestufe die Temperatur und die Zeit des Erhitzens und Haltens innerhalb eines Graphen E'F'G'H' liegen, wobei der Graph E'F'G'H' die Temperatur- und Zeitbereiche darstellt, die durch die Koordinaten von E' (895 °C, 90 s), F' (895 °C, 270 s), G' (940 °C, 210 s) und H' (940 °C, 60 s) definiert sind; und
in der dritten Erhitzungs- und Haltestufe die Temperatur und die Zeit des Erhitzens und Haltens innerhalb eines Graphen I'J'K'L' liegen, wobei der Graph I'J'K'L' die Temperatur- und Zeitbereiche darstellt, die durch die Koordinaten von I' (945 °C, 60 s), J' (945 °C, 240 s), K' (955 °C, 180 s) und L' (955 °C, 30 s) definiert sind.

2. Das Verfahren zur Herstellung eines Heißpräge-Bauteils mit einer Aluminium-Silizium-Legierungsbeschichtung nach Anspruch 1, wobei beim Wärmebehandlungsprozess des Rohlings die Temperatur schrittweise in der Reihenfolge der ersten, zweiten und dritten Erhitzungs- und Haltestufe erhöht wird oder die Temperaturen in der ersten, zweiten und dritten Erhitzungs- und Haltestufe auf bestimmte Temperaturen eingestellt werden.

3. Das Verfahren zur Herstellung eines Heißpräge-Bauteils mit einer Aluminium-Silizium-Legierungsbeschichtung nach Anspruch 1, wobei die Zeit des Wärmebehandlungsprozesses des Rohlings nicht weniger als 150 s und nicht mehr als 600 s beträgt.

4. Das Verfahren zur Herstellung eines Heißpräge-Bauteils mit einer Aluminium-Silizium-Legierungsbeschichtung nach Anspruch 1, wobei ein Wärmebehandlungsofen für den Wärmebehandlungsprozess des Rohlings verwendet wird, der Sauerstoffgehalt in der Ofenatmosphäre nicht weniger als 15 % beträgt und der Taupunkt im Ofen nicht höher als -5 °C ist.

5. Das Verfahren zur Herstellung eines Heißpräge-Bauteils mit einer Aluminium-Silizium-Legierungsbeschichtung nach Anspruch 1, wobei bei dem Heißprägeverfahren der wärmebehandelte Rohling schnell in eine Form zum Prägen überführt wird, die Überführungszeit 4-12 Sekunden beträgt und der Rohling eine Temperatur von nicht weniger als 600 °C aufweist, bevor er in die Form eingeführt wird; die Form vor dem Prägen gekühlt wird, um sicherzustellen, dass die Oberflächentemperatur der Form vor dem Prägen weniger als 100 °C beträgt, und die Abkühlungsgeschwindigkeit des Rohlings größer als 30 °C/s ist.

6. Das Verfahren zur Herstellung eines Heißpräge-Bauteils mit einer Aluminium-Silizium-Legierungsbeschichtung nach Anspruch 1, wobei die mit einer Aluminium-Silizium-Legierungsbeschichtung beschichtete Stahlplatte ein Substrat und eine Aluminium-Silizium-Legierungsbeschichtung auf mindestens einer Oberfläche des Substrats umfasst und das Substrat die folgende Zusammensetzung in Gewichtsprozent umfasst: C: 0,04-0,8 %, Si<1,2 %, Mn: 0,1-5 %, P<0,3 %, S<0,1 %, Al<0,3 %, Ti<0,5 %, B<0,1 %, Cr<3 %, und der Rest Fe und unvermeidliche Verunreinigungen sind.

7. Das Verfahren zur Herstellung eines Heißpräge-Bauteils mit einer Aluminium-Silizium-Legierungsbeschichtung nach Anspruch 6, wobei die Aluminium-Silizium-Legierungsbeschichtung die folgende Zusammensetzung in Gewichtsprozent umfasst: Si: 4-14 %, Fe: 0-4 %, und der Rest Al und unvermeidliche Verunreinigungen ist.

8. Das Verfahren zur Herstellung eines Heißpräge-Bauteils mit einer Aluminium-Silizium-Legierungsbeschichtung nach Anspruch 6 oder 7, wobei das Durchschnittsgewicht der Aluminium-Silizium-Legierungsbeschichtung 58-105 g/m² auf einer Seite beträgt.

9. Das Verfahren zur Herstellung eines Heißpräge-Bauteils mit einer Aluminium-Silizium-Legierungsbeschichtung nach Anspruch 6 oder 7, wobei das Durchschnittsgewicht der Aluminium-Silizium-Legierungsbeschichtung 72-88 g/m² auf einer Seite beträgt.

## Revendications

1. Procédé de fabrication d'un composant d'estampage à chaud ayant un revêtement en alliage aluminium-silicium, comprenant les étapes suivantes : usiner une plaque d'acier revêtue d'un alliage aluminium-silicium, en un flan ayant une forme requise pour une pièce ; procéder au traitement à chaud et à l'estampage à chaud du flan ;
dans lequel, dans le traitement à chaud du flan, le flan est mis dans un four de traitement à chaud pour un traitement d'austénitisation, et le processus de traitement à chaud du flan comprend une premier stade de chauffe et de maintien, un deuxième stade de chauffe et de maintien, et un troisième stade de chauffe et de maintien ;
et dans lequel :
quand l'épaisseur de la plaque d'acier revêtue d'un revêtement en alliage aluminium-silicium est inférieure à 1,5 mm,
dans le premier stade de chauffe et de maintien, la température et le temps de chauffe et de maintien figurent à l'intérieur d'un graphique ABCD, le graphique ABCD représente les plages de température et de temps définies par des coordonnées de A (750°C, 30 s), B (750°C, 90 s), C (870°C, 90 s) et D (870°C, 30 s) ; et
dans le deuxième stade de chauffe et de maintien, la température et le temps de chauffe et de maintien figurent à l'intérieur d'un graphique EFGH, le graphique EFGH représente les plages de température et de temps définies par des coordonnées de E (875°C, 60 s), F (875°C, 240 s), G (930°C, 150 s) et H (930°C, 30 s) ; et
dans le troisième stade de chauffe et de maintien, la température et le temps de chauffe et de maintien figurent à l'intérieur d'un graphique IJKL, le graphique IJKL représente les plages de température et de temps définies par des coordonnées de I (935°C, 60 s), J (935°C, 240 s), K (955°C, 180 s) et L (955°C, 30 s) ; et
quand l'épaisseur de la plaque d'acier revêtue d'un revêtement en alliage aluminium-silicium est de 1,5 mm ou plus,
dans le premier stade de chauffe et de maintien, la température et le temps de chauffe et de maintien figurent à l'intérieur d'un graphique A'B'C'D', le graphique A'B'C'D' représente les plages de température et de temps définies par des coordonnées de A' (750°C, 30 s), B' (750°C, 90 s), C' (890°C, 90 s) et D' (890°C, 30 s) ; et
dans le deuxième stade de chauffe et de maintien, la température et le temps de chauffe et de maintien figurent à l'intérieur d'un graphique E'F'G'H', le graphique E'F'G'H' représente les plages de température et de temps définies par des coordonnées de E' (895°C, 90 s), F (895°C, 270 s), G (940°C, 210 s) et H' (940°C, 60 s) ; et
dans le troisième stade de chauffe et de maintien, la température et le temps de chauffe et de maintien figurent à l'intérieur d'un graphique I'J'K'L', le graphique I'J'K'L' représente les plages de température et de temps définies par des coordonnées de I' (945°C, 60 s), J' (945°C, 240 s), K' (955°C, 180 s) et L' (955°C, 30 s).

2. Procédé de fabrication d'un composant d'estampage à chaud ayant un revêtement en alliage aluminium-silicium comme revendiqué dans la revendication 1, dans lequel dans le processus de traitement thermique du flan, la température augmente par paliers dans cet ordre : premier, deuxième et troisième stades de chauffe et de maintien, ou les températures dans les premier, deuxième et troisième stades de chauffe et de maintien sont fixées pour être des températures certaines.

3. Procédé de fabrication d'un composant d'estampage à chaud ayant un revêtement en alliage aluminium-silicium comme revendiqué dans la revendication 1, dans lequel le temps du processus de traitement thermique du flan n'est pas inférieur à 150 s et pas supérieur à 600 s.

4. Procédé de fabrication d'un composant d'estampage à chaud ayant un revêtement en alliage aluminium-silicium comme revendiqué dans la revendication 1, dans lequel un four de traitement thermique est utilisé dans le processus de traitement thermique du flan, la teneur en oxygène dans l'atmosphère du four n'est pas inférieure à 15 %, et le point de rosée dans le four n'est pas plus élevé que -5°C.

5. Procédé de fabrication d'un composant d'estampage à chaud ayant un revêtement en alliage aluminium-silicium comme revendiqué dans la revendication 1, dans lequel dans le processus d'estampage à chaud, le flan traité à chaud est transféré rapidement dans un moule pour l'estampage, le temps de transfert est de 4-12 secondes, et le flan est à une température qui n'est pas plus basse que 600°C avant d'être amené dans le moule ; le moule est refroidi avant l'estampage afin de garantir que la température de surface du moule avant l'estampage soit plus basse que 100°C, et la vitesse de refroidissement du flan est supérieure à 30°C/s.

6. Procédé de fabrication d'un composant d'estampage à chaud ayant un revêtement en alliage aluminium-silicium comme revendiqué dans la revendication 1, dans lequel la plaque d'acier revêtue d'un alliage aluminium-silicium comprend un substrat et un revêtement en alliage aluminium-silicium sur au moins une surface du substrat, et le substrat comprend la composition suivante en pourcentage par poids : C : 0,04-0,8 %, Si<1,2 %, Mn : 0,1-5 %, P<0,3 %, S<0,1 %, Al<0,3 %, Ti<0,5 %, B<0,1 %, Cr<3 %, et le reste étant Fe et d'inévitables impuretés.

7. Procédé de fabrication d'un composant d'estampage à chaud ayant un revêtement en alliage aluminium-silicium comme revendiqué dans la revendication 6, dans lequel le revêtement en alliage aluminium-silicium comprend la composition suivante en pourcentage par poids : Si : 4-14 %, Fe : 0,4 %, et le reliquat étant Al et d'inévitables impuretés.

8. Procédé de fabrication d'un composant d'estampage à chaud ayant un revêtement en alliage aluminium-silicium comme revendiqué dans la revendication 6 ou 7, dans lequel le poids moyen du revêtement en alliage aluminium-silicium est de 58-105 g/m² sur un côté.

9. Procédé de fabrication d'un composant d'estampage à chaud ayant un revêtement en alliage aluminium-silicium comme revendiqué dans la revendication 6 ou 7, dans lequel le poids moyen du revêtement en alliage aluminium-silicium est de 72-88 g/m² sur un côté.
